

# United States Patent

[19]

Takahashi et al.

[11] 3,714,021

[45] Jan. 30, 1973

[54] **THERMALLY STABLE INSULATING OIL**

[75] Inventors: **Masaaki Takahashi, Tokyo-to; Takashi Yamauchi, Tokyo; Kensuke Okuda, Tokyo; Akira Ito, Tokyo, all of Japan**

[73] Assignee: **Kureha Kagaku Kogyo Kabushiki Kaisha, Tokyo-to, Japan**

[22] Filed: **Oct. 22, 1970**

[21] Appl. No.: **83,232**

[30] **Foreign Application Priority Data**

Oct. 22, 1969 Japan ..... 44/84060

[52] U.S. Cl. ..... **208/14, 208/19, 208/67,  
208/106**

[51] Int. Cl. ..... **C10g 37/06**

[58] Field of Search ..... **208/14, 19**

[56] **References Cited**

**UNITED STATES PATENTS**

|           |         |                       |        |
|-----------|---------|-----------------------|--------|
| 3,252,887 | 5/1966  | Rizzuti .....         | 208/14 |
| 3,406,111 | 10/1968 | Wynkoop et al. ....   | 208/14 |
| 3,462,358 | 8/1969  | Mills et al. ....     | 208/14 |
| 2,846,372 | 8/1958  | Schneider et al. .... | 208/14 |
| 3,095,366 | 6/1963  | Schieman .....        | 208/19 |

*Primary Examiner*—Herbert Levine

*Attorney*—Sughrue, Rothwell, Mion, Zinn & Macpeak

[57] **ABSTRACT**

A thermally stable insulating oil comprising from 95 to 20 percent by volume of a polycyclic naphthenic hydrocarbon and from 5 to 80 percent by volume of a member selected from the group consisting of a polycyclic aromatic hydrocarbon, its lower alkyl derivative and a mixture thereof.

**18 Claims, No Drawings**

## THERMALLY STABLE INSULATING OIL

## BACKGROUND OF THE INVENTION

## 1. Field of the Invention

The present invention relates to an insulating oil having superior thermal stability, and more particularly, it relates to a novel electrical insulating oil comprising a mixture of a polycyclic naphthenic hydrocarbon having two or more rings in the molecule and a polycyclic aromatic hydrocarbon having two or more rings in the molecule.

## 2. Description of the Prior Art

Conventional mineral oil-type insulating oils used hitherto as transformer oils, condenser oils, cable oils, and the like electrical insulating oils, have been prepared from middle-distilled fractions of crude oil after purification thereof by various treatments. Therefore, the performance of the resulting oil varies over a wide range depending upon the kind and nature of the crude oil used, so that the choice of a suitable crude oil has been a matter of great importance in the production of insulating oils.

These known mineral oils, however, have limited thermal stability, i.e., they have a maximum usable temperature of at most about 100°C. Many difficulties have often been encountered when using these mineral oil-type insulating oils in transformers, condensers, cables and like electrical equipment where they are used at a temperature exceeding the above maximum temperature. It is of course possible to improve the thermal stability to a certain extent by resorting to the addition of an oxidation inhibitor and similar additives, but this is rather impractical because the performance of the insulating oil abruptly decreases when the oxidation inhibitor has been used up.

The present invention is based on the discovery that the gas absorption performance of an insulating oil is unexpectedly improved, more so than any other electrical characteristic, and the thermal stability in the presence of oxygen is also greatly enhanced by admixing a polycyclic aromatic hydrocarbon, having two or more rings in the molecule, to a particular hydrocarbon mixture comprising polycyclic naphthenes having two or more rings in the molecule.

The primary object of the present invention is to provide an electrical insulating oil having improved properties.

## SUMMARY OF THE INVENTION

The present invention provides an electrical insulating oil comprising a mixture of from 95 to 20 percent, by volume, of a polycyclic naphthenic hydrocarbon of two or more rings or alkyl derivatives thereof or a mixture thereof, and 5 to 80 percent, by volume, of a polycyclic aromatic hydrocarbon of two or more rings or alkyl derivatives thereof or a mixture thereof.

## DESCRIPTION OF THE PREFERRED EMBODIMENTS

The polycyclic naphthenic hydrocarbons which may be used in this invention include, for example, decalin, perhydrophenanthrene, perhydropyrene, perhydrofluorene, perhydroanthracene, perhydrochrysene, and like cyclic naphthenes having two to five rings, or  $C_8$  or lower, preferably  $C_4$  or lower,

alkyl derivatives thereof or mixtures of two or more such hydrocarbons. Since these mixtures, however, are hardly analyzable at present and usual ring analysis methods are not applicable, an accurate and detailed structure of these compounds has not been determined. However, it is thought that, after observing the results of various molecular weight determining methods and IR, NMR, UV and like spectrum analyses, and of their general properties, as well as the composition of the feed material aromatic oils, the mixture does consist of polycyclic naphthenes.

The insulating oil composition of the present invention substantially comprises a compound having two to four naphthenic rings, and is entirely new.

The general characteristics of the polycyclic naphthenic hydrocarbon are as follows:

|                                                                |               |
|----------------------------------------------------------------|---------------|
| Specific gravity $d_4^{15}$                                    | 0.85-0.99     |
| Refractive index $n_p^{20}$                                    | 1.45-1.60     |
| Viscosity (30°C) cst                                           | 10-40         |
| Hydrogen/carbon atomic ratio<br>(hereinafter indicated by H/C) | 1.75-2.00     |
| Ignition point                                                 | >125°C        |
| Pour point                                                     | -30° to -60°C |

Although it is expected that the oil composition of this invention exhibits higher values of specific gravity and refractive index due to its unique structure than that of conventional mineral oil-type oils, the oil is also far superior in its electrical properties and oxidative stability to those of conventional mineral oil-type oils, the latter having the following properties:

|                                                           |                   |
|-----------------------------------------------------------|-------------------|
| Dielectric constant ( $\epsilon$ ) (80°C)                 | >2.15             |
| Dielectric tangent % $\tan \delta$ (80°C)                 | <0.001            |
| Volumatic resistivity ( $\Omega \cdot \text{cm}$ ) (80°C) | >10 <sup>16</sup> |
| Insulation breakdown voltage KV/2.5mm                     | >60               |
| Total acid value mg, KOH/g                                | <0.001            |
| Corrosivity                                               | 1 A               |
| Thermal stability (120°C-75 hrs)                          |                   |
| Sludge %                                                  | <0.20             |
| Total acid value mg, KOH/g                                | <0.20             |

However, this conventional oil has an inferior gas absorptivity. According to the present invention, this disadvantage has been overcome by the addition of certain polycyclic aromatic compounds to the polycyclic naphthenic hydrocarbon without adversely affecting its inherent electrical properties.

The polycyclic aromatic hydrocarbon employed as the other component in the oil of the present invention includes polycyclic aromatics having from 2 to 4 rings such as, for example, naphthalene, diphenyl, acenaphthene, fluorene, terphenyl, pyrene, chrysene, and  $C_8$  or lower, alkyl derivatives thereof, and mixtures of two or more such compounds. In addition, an aromatic hydrocarbon in which a portion of the ring is saturated with hydrogen, such as acenaphthene, can be used without departing from the scope of the present invention.

The aforesaid aromatic mixture, however, cannot be completely analyzed, but after various physical analysis, gas chromatographic analysis, etc., the polycyclic aromatic structure was confirmed.

The polycyclic aromatic hydrocarbon utilized in the present invention has the following characteristics:

|                             |           |
|-----------------------------|-----------|
| Specific gravity $d_4^{15}$ | 1.00-1.20 |
| Refractive index $n_p^{20}$ | 1.50-1.68 |
| Viscosity (30°C) cst        | 10-25     |
| Pour point                  | <-40°C    |

## Ignition point

The oil composition of the present invention exhibits the following electrical properties and thermal stability:

|                                                        |        |                                       |
|--------------------------------------------------------|--------|---------------------------------------|
| Dielectric constant ( $\epsilon$ )<br>(80°C)           | >150°C | 2.35 - 2.65                           |
| Dielectric tangent (%)<br>$\tan\delta$ (80°C)          |        | 0.001 - 0.03                          |
| Volumetric resistance<br>( $\Omega\text{-cm}$ ) (80°C) |        | $2 \times 10^{14} - 2 \times 10^{16}$ |
| Insulation breakdown<br>voltage KV/2.5mm               |        | 50 - 80                               |
| Thermal stability<br>(125°C - 75 hrs)                  |        | 0.008 - 0.40                          |
| Sludge %                                               |        | 0.05 - 0.60                           |
| Total acid value                                       |        |                                       |

Due to its aromatic structure, the oil of the present invention has an excellent gas absorptivity as well as excellent electrical properties.

The particular polycyclic naphthenic hydrocarbons and the polycyclic aromatic hydrocarbons used in the present invention are easily obtainable by desulfurizing and alkylating (with lower olefins) and/or nuclear hydrogenating bottom oils or tarry materials rich in aromatic compounds, the latter type of material is, for example, formed during the thermal cracking of petroleum hydrocarbons (crude oil, heavy oil, light oil, kerosene, naphtha and the like petroleum fractions) at a temperature of above 700°C but below 2,300°C for a period of time of 1-0.001 second to produce ethylene and/or acetylene, or an oil tar from the gasification of heavy or crude oil at a high temperature, or coal tar, or bottom oil from the dealkylation of alkyl aromatics (e.g., the bottom oil from toluene dealkylation during benzene production).

The desulfurization is conducted employing conventional reaction conditions and conventional catalysts at a temperature of 350°-450°C, a pressure of 20-100 Kg/cm<sup>2</sup>, a hydrogen/high aromatic oil molar ratio of 5-20, and an LHSV of 0.5-2.0. The catalyst which may be employed includes cobalt-molybdenum, nickel-molybdenum, nickel-cobalt-molybdenum, etc., which may be supported on alumina or silica-alumina.

The alkylation is carried out in the presence of a catalyst by admixing a tarry fraction with an olefin gas. The reaction conditions to be employed are as follows:

|                                        |                           |
|----------------------------------------|---------------------------|
| Reaction temperature                   | 250° - 380°C              |
| Pressure                               | 1 - 50 Kg/cm <sup>2</sup> |
| Olefin/tar (molar ratio)               | 0.2 - 10                  |
| Liquid hourly space velocity<br>(LHSV) | 0.1 - 3.0                 |

The catalyst employed in the alkylation may be an acidic catalyst such as silica-alumina, zeolite, etc., but the use of a catalyst in which a Group III-B metal, such as lanthanum, cerium or thorium, is supported on zeolite is especially effective. Under these conditions, the alkylation proceeds smoothly to give the desired product in a good yield.

The degree of alkylation can be controlled to the desired extent by modifying the olefin/tar mixing ratio or liquid hourly space velocity (LHSV).

The electrical properties of the product are not significantly influenced by the type of alkyl group introduced as long as it is not larger than C<sub>4</sub>. Thus, the specific alkyl group employed is determined based on economics, considering the availability of the material. The degree of alkylation is suitably controlled, in

general, to such an extent that the number of alkyl groups attached per average molecular weight of the material aromatic oil ranges on the order of below 5, preferably 1-4, since no substantial fluctuation in the electrical properties of the product can be noticed within this range. A degree of alkylation departing from this range is not desirable from the viewpoint of the yield rather than the electrical properties of the product.

10 The hydrogenation reaction is conducted under conventional conditions employed in the art. Preferred hydrogenation catalysts to be used are exemplified by the oxides, sulfides, etc., of Group VI, VII and VIII metals of the Periodic Table. These catalysts may be supported on carriers such as activated carbon fuller's earth, diatomaceous earth, bauxite, pumice stone, silica-alumina, etc. The reaction is ordinarily conducted at a temperature of 100°-450°C, under a pressure of 10-300 kg/cm<sup>2</sup>, at a liquid hourly space velocity (LHSV) of 0.5-2.0, and at a hydrogen/alkylated high aromatic oil molar ratio of 5-20.

15 The polycyclic naphthenes and polycyclic aromatics should be mixed, according to the present invention, in most cases within a range of 95-20 percent, by volume, of the former to 5-80 percent, by volume, of the latter, although this ratio varies to some extent depending upon the type of electrical equipment to be used. An increased proportion of polycyclic naphthenes beyond the above stated range will result in a decrease in gas absorptivity, and a proportion less than the stated range will cause poorer electrical properties.

20 By mixing both components within the above-mentioned ratio, it is possible to attain remarkable improvements, especially with respect to the gas absorptivity and the voltage pressure resistance among other electrical properties, while still maintaining suitable control of the other properties such as tan  $\delta$ , insulation resistance etc., to appropriate values for given uses. It is surprising that the thermal stability of the mixture in the presence of oxygen can be greatly improved to an extent far superior to that of either of the polycyclic naphthenes or polycyclic aromatics individually.

25 Although each component of the hydrocarbon oil of the present invention itself exhibits excellent electrical performance, it has now been found that surprising effects, which cannot be attained by the use of the conventional mineral type-insulating oil, have been realized by mixing both compounds together.

30 The insulating oil obtained according to this invention has demonstrated outstanding and excellent results, especially when used as a transformer oil, a cable oil and a condenser oil having thermal resistance.

35 The present invention will be further explained by reference to the following non-limiting examples.

## EXAMPLE 1

40 A tarry material obtained by treating Seria crude oil at 1250°C for a contact time of 0.005 second was determined by analysis to have an aromatic distribution comprising 47 percent dicyclic compounds, 33 percent tricyclic compounds, 19 percent tetracyclic compounds and 1 percent pentacyclic compounds, and determined by NMR to have a total of 7 percent side chain hydrogen comprising 4 percent CH<sub>2</sub> and 3 percent CH<sub>3</sub>. This tarry material was desulfurized in a

hydrogen gas stream by using an ordinary desulfurization catalyst consisting of cobalt-molybdenum-alumina, then alkylated with ethylene using silica-alumina as a catalyst to give a polycyclic aromatic hydrocarbon mixture (B).

The mixture (B) had a boiling point (calculated at normal pressure) of 280°-380°C, a composition after type analysis by silica gel absorption comprising 99.1 weight percent aromatics and 0.9 weight percent non-aromatics, and, by Mass spectrometry analysis, comprising 60.1 percent dicyclic rings, 35.4 percent tricyclic rings and 4.5 percent tetracyclic rings.

A portion of (B) was completely nuclear-hydrogenated using a conventional nickel-alumina type catalyst to form a polycyclic naphthenic hydrocarbon mixture (A).

(A) had the following properties: boiling point (calculated at normal pressure) = 290°-370°C, a composition after type analysis by silica gel absorption comprising 2.6 weight percent aromatics and 97.4 weight percent non-aromatics; and by Mass spectrometry analysis comprising 63.2 percent dicyclic rings, 34.2 percent tricyclic rings and 2.6 percent tetracyclic rings.

(A) and (B) were then mixed in a ratio of 75/25, 50/50 and 25/75 by volume, respectively.

The properties and electrical performances of the resulting three compositions are given in Table 1. As is apparent from the table, the characteristics of these mixtures after degradation were found to be very excellent.

TABLE 1

|                                                          | Feed oil A<br>(polycyclic<br>naphthenes) | Feed oil B<br>(polycyclic<br>aromatics) | Thermally stable insulating oil |                      |                      | JIS No. 2 oil<br>(commercial<br>mineral oil) |
|----------------------------------------------------------|------------------------------------------|-----------------------------------------|---------------------------------|----------------------|----------------------|----------------------------------------------|
|                                                          |                                          |                                         | I(A/B = 75/25)                  | II(A/B = 50/50)      | III(A/B = 25/75)     |                                              |
| Specific gravity, $d_4^{15}$                             | 0.983                                    | 1.002                                   | 0.993                           | 0.995                | 1.002                | 0.980                                        |
| Refractive index, $n_p^{20}$                             | 1.504                                    | 1.582                                   | 1.525                           | 1.540                | 1.568                | 1.485                                        |
| Viscosity (est.) 30°C                                    | 24.0                                     | 15.8                                    | 16.2                            | 16.0                 | 15.9                 | 10.5                                         |
| Viscosity (est.) 75°C                                    | 5.4                                      | 4.0                                     | 4.4                             | 4.3                  | 4.1                  | 3.4                                          |
| Pour point, °C                                           | -42.5                                    | -45.0                                   | -42.5                           | -45.0                | -45.0                | -47.5                                        |
| Ignition point, °C                                       | 161                                      | 164                                     | 162                             | 163                  | 163                  | 140                                          |
| Acidic value mg., KOH/g.                                 | 0.003                                    | 0.003                                   | 0.003                           | 0.003                | 0.003                | 0.004                                        |
| Copper plate corrosion, angstroms                        | 1                                        | 1                                       | 1                               | 1                    | 1                    | 1                                            |
| Dielectric constant (80°C)                               | 2.25                                     | 2.65                                    | 2.35                            | 2.40                 | 2.53                 | 2.25                                         |
| tan δ (80°) {Initial}                                    | 0.001                                    | 0.07                                    | 0.01                            | 0.015                | 0.034                | 0.13                                         |
| tan δ (80°) {After degradation*}                         | 0.20                                     | 0.85                                    | 0.08                            | 0.04                 | 0.08                 | 12.2                                         |
| Volumetric resistance (80°C) (Ω-cm.) {Initial}           | $2.0 \times 10^{16}$                     | $6.0 \times 10^{14}$                    | $3.0 \times 10^{15}$            | $1.3 \times 10^{15}$ | $2.0 \times 10^{16}$ | $5.0 \times 10^{13}$                         |
| Volumetric resistance (80°C) (Ω-cm.) {After degradation} | $1.6 \times 10^{14}$                     | $4.0 \times 10^{13}$                    | $2.5 \times 10^{14}$            | $4.0 \times 10^{14}$ | $2.3 \times 10^{14}$ | $2.8 \times 10^{11}$                         |
| Hydrogen gas absorptivity (mm.)**                        | +150                                     | -180                                    | -50                             | -120                 | -160                 | -30                                          |

TABLE 2

|                                                          | Feed oil C<br>(polycyclic<br>naphthenes) | Feed oil D<br>(polycyclic<br>aromatics) | Thermally stable insulating oils |                      |                      |
|----------------------------------------------------------|------------------------------------------|-----------------------------------------|----------------------------------|----------------------|----------------------|
|                                                          |                                          |                                         | IV(C/D = 75/25)                  | V(C/D = 50/50)       | VI(C/D = 25/75)      |
| Specific gravity, $d_4^{15}$                             | 0.942                                    | 1.024                                   | 0.965                            | 0.983                | 1.001                |
| Refractive index, $n_p^{20}$                             | 1.507                                    | 1.605                                   | 1.536                            | 1.560                | 1.582                |
| Viscosity (est.) 30°C                                    | 21.0                                     | 17.4                                    | 20.0                             | 19.0                 | 18.0                 |
| Viscosity (est.) 75°C                                    | 5.2                                      | 4.3                                     | 5.0                              | 4.8                  | 4.4                  |
| Pour point, °C                                           | -43.0                                    | -45.0                                   | -43.5                            | -44.5                | -45.0                |
| Ignition point, °C                                       | 151                                      | 155                                     | 152                              | 152.5                | 153                  |
| Acid value mg., KOH/g.                                   | 0.003                                    | 0.003                                   | 0.003                            | 0.003                | 0.003                |
| Copper plate corrosion, angstroms                        | 1                                        | 1                                       | 1                                | 1                    | 1                    |
| Dielectric constant (80°C)                               | 2.18                                     | 2.60                                    | 2.32                             | 2.40                 | 2.55                 |
| tan δ (percent) (80°) {Initial}                          | 0.001                                    | 0.03                                    | 0.009                            | 0.010                | 0.025                |
| tan δ (percent) (80°) {After degradation*}               | 0.20                                     | 0.35                                    | 0.07                             | 0.03                 | 0.060                |
| Volumetric resistance (80°C) (Ω-cm.) {Initial}           | $4.3 \times 10^{16}$                     | $1.0 \times 10^{15}$                    | $3.5 \times 10^{15}$             | $4.8 \times 10^{15}$ | $6.0 \times 10^{15}$ |
| Volumetric resistance (80°C) (Ω-cm.) {After degradation} | $2.5 \times 10^{14}$                     | $8.0 \times 10^{13}$                    | $7.8 \times 10^{14}$             | $5.0 \times 10^{14}$ | $2.3 \times 10^{14}$ |
| Hydrogen gas absorptivity (mm.)**                        | +140                                     | -180                                    | -40                              | -120                 | -150                 |

\* A copper coil and a 100cc sample of the oil were placed in a 200cc beaker, and the degradation test was carried out for 75 hours in a hot air dryer at 120°C.

\*\* A voltage of 10KV was applied at 80°C under a hydrogen atmosphere, and the gas generation (+) and gas absorption (-) were expressed by an oil manometer.

## EXAMPLE 2

A bottom oil material was obtained as a by-product in the production of ethylene-propylene by the thermal cracking of Kuwait naphtha at 800°C for the contact time of 0.5 second. This bottom oil had an aromatic ring distribution comprising 76 percent dicyclic compounds, 21 percent tricyclic compounds and 3 percent tetracyclic compounds, and total side chain hydrogen of 20 percent comprising 5%  $CH_2$ , 5%  $CH_3$  and 10%  $CH_2-CH_3$  by NMR analysis, which was an aromatic oil containing relatively many side chains.

This oil was desulfurized in a manner similar to that shown in Example 1 to prepare a polycyclic aromatic hydrocarbon mixture (D).

(D) had the following properties: boiling point (calculated at normal pressure) = 280°-380°C, a composition after type analysis by silica gel absorption comprising 99.2 weight percent aromatics and 0.8 weight percent non-aromatics; and by Mass spectrometry analysis comprising 70.5 percent dicyclic rings, 26.8 percent tricyclic rings and 2.7 tetracyclic rings.

This aromatic hydrocarbon mixture (D) was hydrogenated according to a procedure similar to that described in Example 1 to prepare a polycyclic naphthenic hydrocarbon mixture (C).

(C) had the following properties: boiling point (calculated at normal pressure) = 280°-380°C, a composition after type analysis by silica gel absorption comprising 1.8 weight percent aromatics and 98.2 weight percent non-aromatics; and by Mass spectrometry analysis comprising 44.2 percent dicyclic rings, 51.8% tricyclic

rings and 4.0 percent tetracyclic rings.

Both hydrocarbon mixtures (C) and (D) were blended in ratios of 75/25, 50/50 and 25/75 by volume, respectively, to form three examples of the insulating oil of this invention, the properties and electrical per-

formances of which are shown in Table 2.

As is understood from Table 2, the improvement attained by mixing the two components was remarkable.

\* See the note in Table 1.

\*\* See the note in Table 1.

### EXAMPLE 3

The material oil used in this example was a byproduct bottom oil formed in a process for the production of ethylene and propylene were Kuwait naphtha was thermally cracked in a tubular furnace at a reaction temperature of 830°C for the contact time of 0.4 second. This bottom oil was hydrogenated using a nickel-molybdenum-alumina catalyst in the presence of hydrogen at a temperature of 350°C, an LHSV of 0.8 and under a pressure of 40 Kg/cm<sup>2</sup>G. The resulting hydrogenated product was then reacted with 1.5 mole equivalents of propylene in the presence of a silica-alumina type catalyst under a pressure of 10 Kg/cm<sup>2</sup>, an LHSV of 1.0 and at a temperature of 200°C. The oily product was distilled under reduced pressure to give a fraction (E) boiling in the range of 300°-350°C in a yield of 52 percent. This fraction was then determined by mass spectrometry and type analysis by adsorption on silica gel to have the following composition:

|                                         |      |
|-----------------------------------------|------|
| Type analysis by Silica gel adsorption: |      |
| Aromatics weight %                      | 98.5 |
| Non-aromatics weight %                  | 1.5  |
| Mass spectrometry                       |      |
| Dicyclic rings (%)                      | 61.5 |
| Tricyclic rings (%)                     | 37.7 |
| Tetracyclic rings (%)                   | 0.8  |

This fraction (E) was mixed with the polycyclic naphthenic hydrocarbon mixture (C) obtained in Example 2 in ratios of E/C=75/25 and 50/50 by volume, respectively, to prepare two insulating oil compositions. The performances and properties of the oils are given in the following Table 3.

TABLE 3

|                                               | Thermally stable insulating oil VII (E/C=75/25) | Thermally stable insulating oil VIII (E/C=50/50)                             |
|-----------------------------------------------|-------------------------------------------------|------------------------------------------------------------------------------|
| Specific gravity d <sub>4</sub> <sup>15</sup> | 0.982                                           | 0.961                                                                        |
| Refractive index n <sub>D</sub> <sup>20</sup> | 1.570                                           | 1.548                                                                        |
| Viscosity (cst)                               | { 30°C<br>75°C                                  | { 16.3<br>4.0<br>-47.5                                                       |
| Pour point °C                                 |                                                 | 17.2<br>4.1<br>-47.5                                                         |
| Ignition point °C                             |                                                 | 151<br>152                                                                   |
| Acid value mgKOH/g                            | 0.002                                           | 0.002                                                                        |
| Copper plate corrosion                        | 1 A                                             | 1 A                                                                          |
| Dielectric constant (80°C)                    | 2.38                                            | 2.32                                                                         |
| tan δ (%) (80°C)                              | { Initial<br>After de-<br>gradation*            | { 0.029<br>0.05<br>0.04                                                      |
| Volumetric resis-<br>tance (Ω-cm) (80°C)      | { Initial<br>After de-<br>gradation*            | { 1.3 × 10 <sup>16</sup><br>4.8 × 10 <sup>14</sup><br>3.7 × 10 <sup>14</sup> |
| Hydrogen gas absorp-<br>tivity (mm) **        | -100                                            | -60                                                                          |

\* See the note in Table 1.

\*\* See the note in Table 1.

What is claimed is:

1. A thermally stable electrical insulating oil with improved gas absorption performance comprising from 5 to 80 percent by volume of a member selected from the group consisting of one or more polycyclic naphthenic hydrocarbons, lower alkyl derivatives thereof and a mixture of such naphthenic hydrocarbons and lower alkyl derivatives, and from 95 to 20 percent by volume

of a member selected from the group consisting of one or more polycyclic aromatic hydrocarbons, lower alkyl derivatives thereof and a mixture of such aromatic hydrocarbons and lower alkyl derivatives, the polycyclic naphthenic hydrocarbons being obtained by hydrogenating an aromatic fraction which is obtained by the thermal cracking of petroleum hydrocarbons at a temperature above 700°C.

2. The thermally stable insulating oil of claim 1 wherein the one or more polycyclic naphthenic hydrocarbons, lower alkyl derivatives thereof and mixtures thereof, have a specific gravity d<sub>4</sub><sup>15</sup> of from 0.85 to 0.99, a refractive index n<sub>D</sub><sup>20</sup> of from 1.45 to 1.60, a viscosity (30°C.) of from 10 to 40 cst, a hydrogen/carbon atomic ratio of from 1.75 to 2.00, an ignition point of above 125°C., and a pour point of from -30° to -60°C.

3. The thermally stable insulating oil of claim 1 wherein the one or more polycyclic aromatic hydrocarbons, lower alkyl derivatives thereof and mixtures thereof, have a specific gravity d<sub>4</sub><sup>15</sup> of from 1.00 to 1.20, a refractive index n<sub>D</sub><sup>20</sup> of from 1.50 to 1.68, a viscosity (30°C.) of from 10 to 25 cst, an ignition point of above 150°C., and a pour point of below -40°C.

4. The thermally stable insulating oil of claim 1 wherein more than one polycyclic naphthenic hydrocarbon is present as a mixture of polycyclic naphthenic hydrocarbons, each having from two to five rings, their lower alkyl derivatives or a mixture thereof.

5. The thermally stable insulating oil of claim 1 wherein the polycyclic aromatic hydrocarbon is a mixture of polycyclic hydrocarbons each having from two to four rings, their lower alkyl derivatives or a mixture thereof.

6. The thermally stable insulating oil of claim 1 wherein the polycyclic naphthenic hydrocarbons, lower alkyl derivatives thereof and mixtures thereof are obtained by desulfurization, alkylation and hydrogenation of an aromatic fraction which is obtained by the high temperature cracking of petroleum hydrocarbons.

7. The thermally stable insulating oil of claim 6 wherein the alkylation is carried out with butylene, propylene or ethylene.

8. The thermally stable insulating oil of claim 1 wherein the polycyclic aromatic hydrocarbons are obtained by desulfurization and alkylation of an aromatic fraction which is obtained by the high temperature thermal cracking of the petroleum hydrocarbons.

9. The thermally stable insulating oil of claim 8 wherein the alkylation is carried out with butylene, propylene or ethylene.

10. The thermally stable insulating oil of claim 1 wherein the alkyl portion of the lower alkyl derivatives contains less than eight carbon atoms.

11. The thermally stable insulating oil of claim 10 wherein the alkyl portion of the alkyl derivative contains four or less carbon atoms.

12. The thermally stable insulating oil of claim 1 having the following properties:

Dielectric constant (ε) (80°C) 2.35 - 2.65

Dielectric tangent (%) tan δ (80°C) 0.001 - 0.03

Volumetric resistance (Ω-cm) (80°C) 2 × 10<sup>14</sup> - 2 × 10<sup>16</sup>

Insulation breakdown voltage KV/2.5mm 50 - 80

Thermal stability (125°C - 75 hrs)

Sludge % 0.008 - 0.40

Total acid value 0.05 - 0.60.

13. The thermally stable insulating oil of claim 1 wherein the polycyclic hydrocarbons are obtained by desulfurization and alkylation of an aromatic fraction obtained by the high temperature cracking of the petroleum hydrocarbons at a temperature greater than 700°C. to yield the polycyclic aromatic hydrocarbons, and a portion of the polycyclic aromatic hydrocarbons is thereafter hydrogenated to yield the polycyclic naphthenic hydrocarbons, the polycyclic naphthenic and the polycyclic aromatic hydrocarbons thereafter being blended to yield the thermally stable insulating oil.

14. The thermally stable insulating oil of claim 13 wherein the thermal cracking is at a temperature of above 700°C but below 2,300°C for a period of time above from 1 to 0.001 seconds.

15. The thermally stable insulating oil of claim 14 wherein the material cracked is selected from the group consisting of crude oil, heavy oil, light oil, kerosene, naphtha, an oil tar from the gasification of heavy or crude oil at a high temperature, a coal tar or a

bottom oil from the dealkylation of alkyl aromatics.

16. The thermally stable insulating oil of claim 1 wherein the polycyclic naphthenic hydrocarbon is selected from the group consisting of decaline, perhydrophenanthrene, perhydropyrene, perhydrofluorene, perhydroanthracene and perhydrochrysene, alkyl derivatives thereof wherein the alkyl group contains eight or less carbon atoms, and mixtures thereof.

17. The thermally stable insulating oil of claim 1 wherein the polycyclic aromatic hydrocarbon has from 2 to 4 rings and is selected from the group consisting of naphthalene, diphenyl, acenaphthene, fluorene, terphenyl, pyrene, chrysene, alkyl derivatives thereof wherein the alkyl group has eight or less carbon atoms and mixtures thereof.

18. The thermally stable insulating oil of claim 1 wherein the number of alkyl groups attached per average molecular weight of the oil is from 1 to 4.

\* \* \* \* \*

25

30

35

40

45

50

55

60

65